

## UNITED STATES PATENT OFFICE

THOMAS R. SHELTON, OF SAN FRANCISCO, CALIFORNIA, ASSIGNOR OF ONE-HALF TO  
CHARLES A. DOYLE, OF SAN FRANCISCO, CALIFORNIA

## SIZING MATERIAL

No Drawing.

Application filed July 18, 1928. Serial No. 293,789.

This invention relates to sizings and coverings particularly adapted for use on window shades and automobile tops. Such substances should be waterproof, flexible and unaffected by sunlight. The sizings now used for covering window shades comply with neither of these requirements and further than this the application of sizings now in general use are subject to numerous difficulties and objections. For example, since such sizings readily absorb moisture, it is necessary in damp weather that the plants in which such sizing is applied to shades or other materials, be heated, for otherwise it has been found that the sizing absorbs a sufficient amount of moisture to hinder it from properly drying. Again, on days in which the temperature rises above 84° F. it has been found that the sizing ordinarily used evaporates and dries so quickly that it is impossible to properly apply it. This necessitates that the plant be shut down during such weather, and, therefore, materially increases the cost of operation, as likewise does the necessity of heating the plant in damp weather.

In general it is the object of this invention to provide a sizing by which a flexible, weather and water resistant material may be made, and which may be applied under all normal weather conditions.

More specifically, the object of my invention is the provision of a water resistant sizing containing casein, borax, animal glue, para-formaldehyde and tung oil.

The invention possesses other advantageous features, some of which with the foregoing will be set forth at length in the following description. It is to be understood, however, that the scope of my invention is to be limited only by the claims appended to this specification and the prior art.

The sizing of my invention consists of two phases intimately mixed at a temperature of substantially 125° F. It is thinned with water at this same temperature to any desired consistency and heated to a temperature of substantially 135° F. for application to shade or other materials.

The first phase is made as follows:—Two gallons of China wood or tung oil are treated

to a temperature of 550° F. The oil so treated is then mixed with ten pounds of eighty mesh casein, eight and a quarter pounds of borax, and one ounce of para-formaldehyde. This mixture is then continuously stirred with the addition of water at a temperature of substantially 125° F. in a sufficient amount to absorb the mixture to form a thick paste. When this paste has been stirred to a uniform consistency, it is allowed to stand for several hours, approximately three. At the end of this time an exothermic chemical reaction will be found to have taken place and due to its exothermic character the temperature of the paste will be found to be approximately 125° F.

The second phase of my sizing is made up while the first phase or paste is being allowed to stand and is made as follows:—Twenty-three pounds of hide glue and thirteen pounds of bone glue are mixed with and allowed to absorb five gallons of cold water. This process should not take longer than three or four hours. After having allowed the glue to stand for several hours it is heated to a temperature of approximately 125° F. Needless to say, both hide and bone glue are of the animal variety. The hide glue used corresponds very closely with what is known as No. 11 or 12 standard glue, while the bone glue corresponds very closely with what is known as No. 2 standard glue.

The first phase (the thick paste formed by the casein, borax, formaldehyde and tung oil) is then added to the second phase (animal glue). This addition as above stated takes place at a temperature of approximately 125° F. The resulting sizing can then be thinned to any desired consistency for application. It has been found that about fifty-six gallons of sizing will be produced by the various ingredients mixed in the quantities as above stated.

The action of borax and formaldehyde on the casein seems to be more or less generally understood and other suitable materials to aid in the dissolving and hardening of the casein can be used. It has been found the proportions of all of the ingredients used are rather critical and cannot therefore be varied.

to any great extent for the substance named. Likewise the temperatures used have been found critical. The flexibility of the sizing is attributed to the tung oil which also acts as a drying oil but no attempt is made to give the chemical reaction taking place between this substance and the other substances forming the sizing. The use of tung oil seems to be entirely new for this purpose.

10 The final product appears to be irreversible and although it is known that formaldehyde reacts with casein to make the casein jelly irreversible, as far as the applicant is aware this has never before been done with an animal glue.

15 Shades covered with a sizing made up according to the above recipe are found to be waterproof, unaffected by sunlight and capable of being bent and creased without any apparent injury. Furthermore, it has been found out that this sizing will not absorb water and therefore may be applied just as readily in damp weather as in dry weather. The rate of evaporation is sufficiently low to permit of its being readily applied at atmospheric temperatures well above 84° F.

I claim:

1. A water resistant sizing containing the following ingredients in substantially the proportions stated: two gallons of tung oil, ten pounds of casein, eight pounds of borax, one ounce of para-formaldehyde and thirty-six pounds of animal glue.

2. A water resistant sizing containing the following ingredients in substantially the proportions stated: two gallons of tung oil, ten pounds of casein, eight pounds of borax, one ounce of para-formaldehyde, twenty-three pounds of hide glue and thirteen pounds of bone glue.

3. The process of making a water resistant sizing comprising the following steps:— mixing heat treated tung oil with casein, borax, formaldehyde and water to form a thick paste, allowing the paste so formed to stand for several hours; adding a hot, water soaked animal glue to said paste and in then thinning the mixture so formed with water to any desired consistency for application.

4. The process of making a water resistant sizing comprising the following steps; mixing heat treated tung oil with casein, borax, formaldehyde and water to form a thick paste; allowing the paste so formed to stand for several hours; adding said paste to a hot water soaked animal glue and in then thinning the mixture so formed with water to any desired consistency for application.

5. The process of making a water resistant sizing comprising the following steps; mixing two gallons of heat treated tung oil with ten pounds of casein, eight pounds of borax soap chips, one ounce of para-formaldehyde and sufficient water to form a thick paste; al-

lowing the paste so formed to stand for several hours; adding said paste to thirty-six pounds of animal glue soaked in five gallons of water and in then thinning the sizing so formed with water to any desired consistency for application.

6. The process of making a water resistant sizing comprising the following steps; mixing heat treated tung oil with casein, borax, formaldehyde and hot water to form a thick paste; allowing the paste so formed to stand for several hours; adding to said paste a water absorbed animal glue at a temperature of substantially 125° F. and in then thinning the sizing so formed with water at substantially 125° F. to any desired consistency for application.

7. The process of forming a water resistant sizing comprising adding a mixture of tung oil, casein, borax and formaldehyde, when at a temperature of approximately 125° F. to a liquid mass of water-soaked animal glue when at a substantially similar temperature and then thinning the mixture thus formed by the addition of water heated to substantially the same temperature.

In testimony whereof, I have hereunto set my hand.

THOMAS R. SHELTON.

95

100

105

110

115

120

125

130

70

75

80

85

90

95

100

105

110

115

120

125

130